

April 22, 1952

W. B. COLEMAN ET AL  
SINGLE-BATH CHROME DYEING PROCESSES AND  
COMPOSITIONS, INCLUDING AMMONIUM  
SULFATE AND DIAMMONIUM PHOSPHATE  
Filed Oct. 8, 1949

2,593,850



Inventions:  
William B. Coleman,  
Gerald N. Cote,  
By Schroeder Merriman,  
Hofmann Brady, et al.

## UNITED STATES PATENT OFFICE

2,593,850

SINGLE-BATH CHROME DYEING PROCESSES  
AND COMPOSITIONS, INCLUDING AMMO-  
NIUM SULFATE AND DIAMMONIUM PHOS-  
PHATE

William B. Coleman, Crete, Ill., and Gerald M. Coté, Wellesley, Mass., assignors to Victor Chemical Works, a corporation of Illinois

Application October 8, 1949, Serial No. 120,384

11 Claims. (Cl. 8—30)

1

This invention relates to an improvement in chrome dyeing and compositions for use therein.

Chrome dyeing has conventionally been carried out in baths containing Glauber's salt and ammonium sulfate, in addition to the chromate salt and the dye. In the treatment of wool with such baths, the practice has been to prepare a slightly alkaline bath in which the wool is immersed for a sufficient time to swell the fibres and permit penetration by the dyestuffs. Without such alkaline soaking, dyeing occurs merely on the surface. After the alkaline treatment it has been the practice to add successive additions of such acids as formic, acetic, sulfuric and phosphoric to increase the acidity and lower the pH. During this acidification, according to present theories, the wool first reacts with the acid, the acidic wool then combines with the dye, and the dyed wool reacts with the chrome mordant to fix the dye on the wool as an insoluble complex. Metachrome dyeing is a procedure in which both the dye and the chrome mordant are initial components of the dye bath, and the dyeing is controlled by addition of acids at the critical stages of the process.

Normally the application of heat accelerates the dyeing process so that it is conventional to boil the liquid in the bath.

In order to obtain a completely satisfactory chrome dyeing of woolen materials, it is essential that the pH of the bath be very closely controlled. The increase in acidity must be gradual, otherwise, the dye will suddenly deposit upon the fabric, and great unevenness of dyeing will result. Such unevenness is known as "unlevelness" and "skitteriness" in the trade, and is a result of the characteristics of the fibres and a sudden change in pH of the dye bath. A final pH of 5.2 to 5.8 is desired to fully develop and fix the color.

The control of the acidity of the dye bath by addition of acid has several considerable disadvantages. Perhaps the most important is the fact that the bath must be cooled before the acid is added. After this the bath is reheated. This results in a very considerable loss of time, as well

2

as the cost of the heating operation. Secondly, it is quite difficult to control the acidity throughout the solution, particularly since any addition of acid must be made more or less locally, with the result that the pH in that locality is reduced below the general average. Therefore, unlevelness and skitteriness are common.

10 We have discovered that a chrome dyeing bath may be prepared having an initial pH within the desirable range of alkalinity which, by the application of heat may be converted at the desired rate to a bath having an acid pH which will maintain itself automatically in the desired range. Because the change in pH comes from inside the 15 bath, rather than from outside additions, the change can be made with absolute uniformity.

20 These results may be accomplished by the addition to the bath of suitable proportions of diammonium phosphate, or a mixture of diammonium phosphate with one or more ammonium salts of a strong acid, and particularly ammonium sulfate. The initial pH of such a bath is slightly alkaline, but after the bath is heated to boiling, the diammonium phosphate slowly decomposes, resulting 25 in a gradual increase in the acidity of the solution and a gradual deposition of dyestuff upon the fibres. The decomposition of diammonium phosphate proceeds until equilibrium conditions are reached at a pH of 6.2 to 6.5. When diammonium phosphate by itself is used as a buffering agent, the final pH attained by the chrome bath will not drop to below 6.2. Certain colors are developed in a bath of that acidity; however, for other colors an end pH of 5.2 to 5.8 is desirable 30 for full development of the dye. Consequently when a pH of about 6.2 is reached in the dye bath, formic, phosphoric, sulfuric or acetic acid may be added to reduce the final pH to the desired value of 5.2 to 5.8, and the dyeing operation 35 completed at that acidity.

40 The addition of an ammonium salt of a strong acid, as ammonium sulfate, together with diammonium phosphate to a metachrome dye bath, depending upon proportions used, will result in a 45 bath that is initially alkaline, but upon boiling

together with the material to be dyed, will attain the desired pH of 5.2 to 5.8 without the addition of acid. Ammonium sulfate itself does not give the initial alkalinity, and it is added for reasons of producing a final acidity greater than that of diammonium phosphate when used alone. Woolen materials dyed by use of such a bath have resulted in good bath exhaustion, level and full development of bright and fast colors, whereas when a standard metachrome dye bath and methods known to prior art were used, uneven dyeing of cloth was often obtained.

For comparative purposes two chrome dyeing tests were made using: (A) a standard metachrome dye bath of the formula—

2% Chromate Brown EBC dye  
10% Glauber's salt  
3% Ammonium sulfate  
1% Neutral sodium chromate

and, (B) a similar bath in which the 3% ammonium sulfate was replaced with 3% diammonium phosphate. In both cases the percentages are based on the weight of goods to be dyed. The ratio of water to goods was 30 to 1 in both cases. The goods tested were strips of a piece of wool cloth which had been previously "carbonized" in a dilute sulfuric acid bath in accordance with standard commercial practice. The cloth, joined in the form of a continuous belt, was immersed in the dye bath and slowly turned to achieve even wetting of the cloth. The bath was brought to a boil in one hour, and then boiled for an additional forty-five minutes. Two percent (2%) (on weight of cloth) of 28% acetic acid was then added, and the bath boiled an additional half hour.

The following table shows the pH values of the bath at intervals during the operation of the process:

|                              | Bath before contact with wool<br>Room temp. | Bath after contact with wool<br>Room temp. | 15<br>Mins. | 30<br>Mins. | 40<br>Mins. | Start of boil |             |             | Acid addition |              |              | I | II |
|------------------------------|---------------------------------------------|--------------------------------------------|-------------|-------------|-------------|---------------|-------------|-------------|---------------|--------------|--------------|---|----|
|                              |                                             |                                            |             |             |             | 60<br>Mins.   | 75<br>Mins. | 90<br>Mins. | 105<br>Mins.  | 120<br>Mins. | 135<br>Mins. |   |    |
| A. Ammonium sulfate.....     | 7.0                                         | 6.6                                        | 5.2         | 5.7         | 6.2         | 6.4           | 6.4         | 6.4         | 6.4           | 5.1          | 5.1          |   |    |
| B. Diammonium phosphate..... | 7.7                                         | 7.4                                        | 7.1         | 7.1         | 7.1         | 7.1           | 6.7         | 6.7         | 6.7           | 5.4          | 5.4          |   |    |

The influence of the wool acidity can be clearly seen not only at the moment of contact with the bath, but at succeeding intervals as well. The relative stabilities of the solutions toward change are also evident. It will be seen that the standard dye bath formula has little buffering power, whereas the dye bath containing the diammonium phosphate had excellent buffering power. The initial development of acidity in (A) resulted in rapid deposition of the dye on the cloth before a uniform distribution of the dye could take place, whereas the much longer period of alkalinity control in (B) permitted the uniform distribution of dye throughout the cloth before the acidity was increased sufficiently to cause deposition of the dye. The results were that the cloth of test (A) was dyed unevenly, and that of (B) was uniform and highly satisfactory.

As illustrated in the above example (B), the use of a single addition of acid at the end of the boiling period to reduce the final pH gives satisfactory results. This represents an improvement over prior chrome dyeing procedures

where several adjustments in the pH of the bath are necessary to obtain satisfactory results.

By the substitution of ammonium sulfate for the Glauber's salt of the prior art, and the simultaneous use of diammonium phosphate, it has been possible to control the pH of the dye bath from the slight alkalinity required at the start to the low pH of 5.2 to 5.8 desired at the end of the process for fixing the dye, such control being obtained without intermediate adjustments or acid additions.

By use of such new combination of assistants we have found that the dye, mordant and assistants can be employed in a single bath to give an efficient, satisfactory and substantially fool-proof one-step process for the chrome dyeing of wool.

In some cases it may be desirable to adjust the initial pH value of the bath, depending on the nature of the wool to be dyed. For example, the bath may be adjusted with ammonia to offset the acidity of some types of wool, especially those which have had an acid pretreatment.

The one-step dye bath of the present invention should include a predetermined amount of the desired chrome dye with sufficient sodium or ammonium chromate or dichromate to act as a mordant, ammonium sulfate and diammonium phosphate dissolved in water to give a solution of the desired concentration.

Two metachrome dye baths illustrating the invention were made up in the following proportions:

|                               | Per cent | Per cent | I        | II       |
|-------------------------------|----------|----------|----------|----------|
|                               |          |          | Per cent | Per cent |
| Chrome Fast Blue BX Conc..... | 1.0      | 1.0      |          |          |
| Ammonium Sulfate.....         | 20.0     | 30.0     |          |          |
| Diammonium phosphate.....     | 5.0      | 5.0      |          |          |
| Sodium dichromate.....        | 1.0      | 1.0      |          |          |

where percentages refer to weight of wool. The baths were diluted with thirty parts of water per part of cloth. Test dyeings were carried out in these baths and the following conditions noted:

|                                                           | 7.3 adjusted to 7.8 with NH <sub>4</sub> OH. | 7.1 adjusted to 7.8 with NH <sub>4</sub> OH. | I        | II  |
|-----------------------------------------------------------|----------------------------------------------|----------------------------------------------|----------|-----|
|                                                           |                                              |                                              | 7.4..... | 7.5 |
| 60 Bath pH before contact with wool.<br>Room temperature. |                                              |                                              |          |     |
| Bath pH after contact with wool.<br>Room temperature.     |                                              |                                              |          |     |
| Bath pH heated at 180° F.:                                |                                              |                                              |          |     |
| 15 min.....                                               | 7.0                                          |                                              | 7.1      |     |
| 30 min.....                                               | 6.7                                          |                                              | 6.5      |     |
| 45 min.....                                               | 6.5                                          |                                              | 6.3      |     |
| 60 min.....                                               | 6.3                                          |                                              | 6.1      |     |
| 75 min.....                                               | 6.2                                          |                                              | 5.9      |     |
| 90 min.....                                               | 6.0                                          |                                              | 5.8      |     |
| 105 min.....                                              | 5.9                                          |                                              | 5.7      |     |
| 120 min.....                                              | 5.9                                          |                                              | 5.6      |     |
| 135 min.....                                              | 5.8                                          |                                              | 5.5      |     |
| 150 min.....                                              | 5.7                                          |                                              | 5.5      |     |
| 165 min.....                                              | 5.7                                          |                                              | 5.4      |     |

These two compositions gradually reach the desired final pH. The initial pH can be easily adjusted to alkalinity by addition of ammonium

hydroxide at the beginning. Once this adjustment has been made, no additional adjustment is necessary. A buffering action is then obtained that controls the pH of the bath at every level and eliminates fluctuations. Level dyeing, good bath exhaustion, full development of dye and fastness of color were obtained; also the feel of the cloth was satisfactory in both of the above experiments.

The chrome fast blue BX concentrate was chosen in the above examples because it is a dye with which levelness is obtained only by careful control of pH conditions. Chrome Brown EBC, Brown PG, Chrome Orange R Conc., Chrome Fast Violet B, Chrome Green B, Conc., and Chrome Fast Grey G. L. were satisfactorily used. The mordants used have been sodium chromate, sodium dichromate and ammonium chromate. When ammonium chromate was used as the mordant, it was possible to reduce the amount of ammonium sulfate necessary to produce the desired final pH value. However, sodium chromates are preferred because of their commercial availability.

Considerable variation in the amounts and proportions of the assistant compounds is possible without detrimental effect in the dyebath. In general, the proportions are selected to provide a buffered pH range from about 7.5 down to about 5.2. In all cases the pH of the bath will be affected by the type of water used and the condition of the wool; i. e., if the water is hard or soft, and whether the wool is neutral, basic or acidic. To meet conditions that are often encountered in commercial dyeings, such as the necessity of using hard water and/or the use of not completely neutralized wool, it has been found that from 15 to 30% ammonium sulfate, and from 1 to 9% diammonium phosphate with 1 to 3% sodium dichromate (or sodium or ammonium chromates) based on the weight of the wool, will give entirely satisfactory results when employed with 1 to 3% of a chrome dye selected from the class of dyes classified in the A. A. T. C. C. Technical Manual and Year Book of 1947-1948 as "Mordant Acid" dyes, which dyes are capable of forming metallic complexes with a metallic salt, for example, sodium dichromate. When more ideal conditions for dyeing are present, such as soft water and a completely neutralized wool, the amount of ammonium sulfate may be considerably reduced. In such cases good pH control and successful dyeings have been effected with the use of but 10% ammonium sulfate.

It is preferred to prepare the new dye assistant composition as a dry solid material which may be added to the dye bath in the desired concentration, together with the dye selected to give the required color and shade. The function of the mordant compound is that of forming a metal complex with the dye to fix the dye on the wool fibers. The amount of mordant is more or less dependent on the amount of dye employed and the amount of wool being processed, and has no critical relationship to the amounts of ammonium sulfate and diammonium phosphate in the solution or dry composition. In general, the amount of mordant compound should be within the range of 1 to 3% based on the weight of wool to be dyed. The functions of the ammonium sulfate and diammonium phosphate are dependent on each other, and the combination effect is that of buffering the solution over wide range of pH control. In general the higher the proportion of

ammonium sulfate, the lower the pH obtained may be controlled, provided sufficient diammonium phosphate is present to buffer the solution in the higher pH range and control the rate of lowering the pH. We have found that a range of 15 to 30% ammonium sulfate and 1 to 9% of diammonium phosphate, based on the weight of wool, is sufficient for satisfactory pH control of the dye bath. Based on these proportions, a solid composition within the range of 96.7-62.5% ammonium sulfate and from 3.3-37.5% diammonium phosphate will give satisfactory pH control when dissolved in the dye bath.

The drawing is a triaxial diagram illustrating the preferred limits of the three element solid composition. As is well known, the proportion of each ingredient is indicated by that percentage of the distance from the base opposite the indicated 100% point for that compound, to that point. Thus the line AB on the diagram is 93.8% from the base of the triangle to the peak marked 100% ammonium sulfate, and, therefore, indicates 93.8% ammonium sulfate in the composition. The line BC is 2½% of the distance from the base to which it is parallel to the lower left-hand corner representing 100% mordant salt, and therefore indicates 2½% of that material.

The three component solid composition may be made up by mixing the three components in the percentage proportions represented within the area bounded by the lines AB, BC, CD, DE, EF and FA of the triaxial diagram, wherein lines AB and DE define maximum and minimum amounts of ammonium sulfate; lines EF and BC define maximum and minimum amounts of mordant salt; and the lines CD and FA define maximum and minimum amounts of diammonium phosphate. The maximum and minimum amounts of each component are represented by the percentage figures: 93.8-55.6% for ammonium sulfate, 36.0-3.0% for diammonium phosphate and 15.8-2.5% for the mordant salt.

Compositions within the indicated area of the diagram may vary somewhat in their pH control characteristics, but all are capable of effecting a satisfactory control of the dye bath within the pH range of about 7.5 down to about 5.2 during the boiling operation.

Some variation may be encountered in the utilization of such compositions due to the different acidities of the various mordant compounds. It is, therefore, desirable, in addition to the limitations already prescribed for these compounds, to correlate the proportions of the ingredients so that the resulting compound will produce a pH from approximately 6.9 to 7.5 when dissolved in a 1% solution in water. However, as pointed out, if the pH is too low, it may readily be adjusted by the addition of a very small amount of ammonium hydroxide.

The solid compositions represented above may be dissolved in water in concentrations suitable for the dyeing operation. We have found that based on the preferred use of 15 to 30 pounds of ammonium sulfate per 100 pounds of wool, the above assistant compositions may be dissolved in 2000 to 4000 pounds of water, preferably 3000 pounds of water. This means an ammonium sulfate concentration of from 0.375% to 1.5%, preferably from 0.5% to 1.0%. Thus, the solid assistant compositions may be used in the dye bath on the basis of an ammonium sulfate concentration of 0.37 to 1.5% for satisfactory dyeing operations.

As further examples of the invention, dyeings were made using various concentrations and proportions as shown in the following table:

| Assistant Composition                | C       | D       | E       | F       | G       |
|--------------------------------------|---------|---------|---------|---------|---------|
| Dry basis:                           |         |         |         |         |         |
| Ammonium Sulfate.....percent         | 55.5    | 62.5    | 83.3    | 81.1    | 90.0    |
| Diammonium Phosphate.....do          | 33.3    | 31.3    | 12.5    | 13.5    | 6.25    |
| Sodium Dichromate.....do             | 11.2    | 6.2     | 4.2     | 5.4     | 3.75    |
| Total.....do                         | 100.0   | 100.0   | 100.0   | 100.0   | 100.0   |
| Bath—Pounds per 100 pounds of wool:  |         |         |         |         |         |
| Ammonium Sulfate.....                | 15.0    | 10.0    | 20.0    | 30.0    | 24.0    |
| Diammonium phosphate.....            | 9.0     | 5.0     | 3.0     | 5.0     | 1.66    |
| Sodium Dichromate.....               | 3.0     | 1.0     | 1.0     | 2.0     | 1.0     |
| Water.....                           | 3,000.0 | 3,000.0 | 3,000.0 | 3,000.0 | 3,000.0 |
| Dye.....                             | 1.0     | 1.0     | 1.0     | 1.0     | 1.0     |
| Initial pH of bath.....              | 7.0     | 7.3     | 7.1     | 6.9     | 6.7     |
| pH after adding wool.....            | 6.8     | 7.0     | 6.95    | 7.5     | 6.6     |
| After heating 15 min. at 180° F..... | 6.6     | 6.6     | 6.7     | 7.0     | 6.5     |
| 30 min.....                          | 6.3     | 6.5     | 6.4     | 6.5     | 6.3     |
| 45 min.....                          | 6.2     | 6.3     | 6.15    | 6.2     | 6.0     |
| 60 min.....                          | 6.05    | 6.1     | 6.0     | 6.0     | 5.9     |
| 75 min.....                          | 5.9     | 6.0     | 5.9     | 5.9     | 5.75    |
| 90 min.....                          | 5.8     | 5.9     | 5.8     | 5.75    | 5.6     |
| 105 min.....                         | 5.75    | 5.85    | 5.7     | 5.65    | 5.6     |
| 120 min.....                         | 5.7     | 5.8     | 5.7     | 5.6     | 5.5     |
| 135 min.....                         | 5.6     | 5.8     | 5.6     | 5.5     | 5.5     |
| 150 min.....                         | 5.5     | 5.8     | 5.6     | 5.5     | 5.5     |

<sup>1</sup> Adjusted to 7.8 with NH<sub>4</sub>OH.

Dyeing results obtained in examples C, D, E and F were excellent. Those obtained in example G were good.

Example G, while still illustrating an operable procedure, is not so satisfactory as examples C, D, E and F because of the lower buffering capacity at the start of the dyeing operation.

The solid assistant compositions may also include the chrome dyestuff if desired, but it is preferred not to include the dye in order to permit the dye bath operator to standardize on the assistant composition and vary only the dyestuff to obtain the desired colors and shades.

While the above assistant compositions offer a simple and trouble proof means of controlling the dyeing operation, it is sometimes desirable, as in "top chrome" dyeing, to add the mordant salt at a late stage of the dyeing operation. Dyeing operations of this type may be carried out by employing an assistant composition containing the ammonium sulfate and diammonium phosphate, adding the dyestuff and boiling until the desired pH value is reached, then adding the mordant salt.

The foregoing detailed description is given for clearness of understanding only, and no unnecessary limitations should be understood therefrom, as modifications will be obvious to those skilled in the art.

We claim:

1. A dye bath assistant composition consisting of ammonium sulfate, diammonium phosphate and a chromium mordant compound selected from the group consisting of sodium chromate, sodium dichromate, ammonium chromate and ammonium dichromate, wherein the components are selected within the percentage range of 55.6 to 93.8 parts by weight ammonium sulfate, 3.0 to 36.0 parts by weight of diammonium phosphate, and 2.5 to 15.8 parts by weight of the mordant compound.

2. A dye bath assistant composition consisting of ammonium sulfate, diammonium phosphate and a chromium mordant compound selected from the group consisting of sodium chromate, sodium dichromate, ammonium chromate and ammonium dichromate, wherein the components are selected within the percentage range of 55.6 to 93.8 parts by weight ammonium sulfate, 3.0 to

36.0 parts by weight of diammonium phosphate, and 2.5 to 15.8 parts by weight of the mordant compound, and which when dissolved in a 1%

aqueous solution has an initial pH of 6.9 to 7.5 before heating.

3. A composition as set forth in claim 1 in which the mordant is sodium dichromate.

4. A dye bath comprising an aqueous solution including a chrome mordant acid dye, ammonium sulfate, diammonium phosphate and a chromium mordant compound selected from the group consisting of sodium chromate, sodium dichromate, ammonium chromate and ammonium dichromate, wherein the components other than water are selected within the percentage range of 55.6 to 93.8 parts by weight of ammonium sulfate, 3.0 to 36.0 parts by weight of diammonium phosphate, and 2.5 to 15.8 parts by weight of the mordant compound.

5. A dye bath as set forth in claim 4 in which the mordant is sodium dichromate.

6. A dye bath as set forth in claim 4 in which the concentration of ammonium sulfate in the aqueous solution is from 0.37 to 1.5% by weight.

7. A dye bath assistant composition comprising a mixture of ammonium sulfate and diammonium phosphate, the proportions being within the range of 62.5 to 96.7 parts by weight of ammonium sulfate and 37.5 to 3.3 parts by weight of diammonium phosphate.

8. A dye bath composition comprising an aqueous solution containing approximately 1% by weight of ammonium sulfate, 0.17% diammonium phosphate, 0.034% sodium dichromate and a suitable amount of a chrome mordant acid dye.

9. A dye bath assistant composition consisting of approximately 83% by weight ammonium sulfate, 14% diammonium phosphate and 3% of sodium dichromate.

10. The process of dyeing wool which comprises immersing said wool in an aqueous bath containing, per 100 pounds of wool, from 1 to 3 pounds of a chrome dye, from 15 to 30 pounds of ammonium sulfate, from 1 to 9 pounds of diammonium phosphate, and 1 to 3 pounds of a mordant compound selected from the group consisting of sodium chromate, sodium dichromate, ammonium chromate and ammonium dichromate, and heating the bath at a temperature of 180° F. to boiling for a sufficient period to effect automatic lowering of the pH value to within the

range of pH 5.2 to 5.8 without the addition of an acid.

11. The process of dyeing wool which comprises immersing said wool in an aqueous bath containing, per 100 pounds of wool, from 1 to 3 pounds of a chrome dye, from 15 to 30 pounds of ammonium sulfate, from 1 to 9 pounds of diammonium phosphate, and 1 to 3 pounds of a mordant compound selected from the group consisting of sodium chromate, sodium dichromate, ammonium chromate and ammonium dichromate, and heating the bath at a temperature of 180° F. to boiling for a sufficient period to effect automatic lowering of the pH value to within the range of pH 5.2 to 5.8 without the addition of an acid, said bath containing sufficient water to give

a bath weighing from 20 to 40 times the weight of the wool.

WILLIAM B. COLEMAN.  
GERALD M. COTÉ.

#### REFERENCES CITED

The following references are of record in the file of this patent:

10 "Bleaching, Dyeing and Chemical Technology of Textile Fibers," by Trotman and Trotman, 2nd edition, 1946, Griffin and Company, Ltd., London; pages 362 and 363.

15 Amer. Dyestuff Reporter for August 23, 1948, pages P547, P548.

Journal Soc. Dyers and Col. for December 1945, pages 328 to 333.